

June 2, 1936.

H. VON BRANDT

2,042,917

HIGH CONCENTRATION AGAR-AGAR GEL AND COMBINATIONS THEREOF

Filed July 22, 1932



INVENTOR.  
HENRY VON BRANDT.

BY

*Rudolf H. Gruenauer*

ATTORNEY.

## UNITED STATES PATENT OFFICE

2,042,917

HIGH CONCENTRATION AGAR AGAR GEL  
AND COMBINATIONS THEREOF

Henry von Brandt, New York, N. Y.

Application July 22, 1932, Serial No. 624,119

13 Claims. (Cl. 18—47)

This invention concerns a high concentration homogeneous agar agar gel as a base for an imprint material,—and a method of making the same,—more particularly a material serving to obtain a negative imprint of the shape of a plastic body, be it a sculpture, an art object, or a commercial article, a fossil, or a live or dead organic body.

This material finds a prominent use in the arts and in the medical sciences, where a true replica of the human body or any part thereof, like the ear or foot, is to be made. Thus for instance, the dentist may use the material of my invention, where he desires to obtain an imprint of the oral cavity, and in the following exemplary description I have specific reference to an adaptation of my invention for such purposes, although it is understood, that the material as described as well as more or less concentrated may serve in ramified uses.

The grade of concentration as well as the grade of consistency depend largely upon the nature of the object of which an imprint is to be taken. For instance, if a true replica of the dental cavities of a jaw are desired—which case the dental tray filled with the imprint material may have to be turned upside-down in order to be applied—the imprint material should be more concentrated and denser than for taking a delicate imprint, of hair and the like, for instance.

One object of this invention is to prepare an imprint material, which sets quickly while the imprint is being taken, said imprint material showing however sufficient resiliency after the setting, so that it may be removed from the original, for instance a jaw, which shows undercuttings as in dental cavities, the resilient parts of the material being temporarily stretched during removal, while slipping away from such undercuttings.

It is however understood that the material must resume exactly the same shape it had before, after having been withdrawn over the protruding parts and must then retain its shape and size. In other words, it must be truly elastic and resilient and should not remain distorted.

Another object of this invention is to prepare an imprint material in such a manner, that it may be preserved indefinitely, and so that only a short process is required to place it into condition to take an imprint whenever desired.

A further object of this invention is to provide an imprint material, which preserves its exact shape and dimensions for a reasonable length of

time after the imprint has been taken so that true casts may be made therefrom.

Furthermore provisions have been made that the imprint may be preserved, and may be reduced at a later date to the exact size which it had at the time the imprint was taken, a simple process being required thus to re-condition the imprint.

Provisions have also been made whereby it is possible to preserve the exact dimensions, shape and detail of a fresh imprint for larger periods of time without whole or partial losses due to shrinkage, bacterial growth, or mold; this is accomplished by one single, lasting treatment.

Another object of this invention has reference to hygiene. Throughout the whole manufacturing process this imprint material or any part thereof does not require the touch of human hands. The product is sterile, and until the very time of actual use I preserve the material in its original sterile condition.

A further object of this invention is to create an imprint material of white—or very light—color, which may be colored to any desired shade.

It is a very important object of this invention, and one which largely influences the choice of the ingredients, that the material, after an imprint has been taken, may be exposed to any atmosphere without putrefaction or molding.

It is also an object of this invention to allow close control of the setting speed and temperature.

It is further understood that a material of this kind must comprise a binder which holds it together, so that it does not readily break apart; at the same time the material should not be mucilaginous to the extent of adhering to the articles of which an imprint is to be taken; I have reached the object of obviating the covering of the article of which an imprint is to be taken with a coat of material which prevents adhesion of the imprint material to said article. On the other hand the material is to show the greatest possible cohesion.

In order to obtain these various objects and others, which will be further understood from the following, I have not only brought about improvements as to the ingredients used in my material, but I have also developed special and economical processes of preparing the material, and the binder used therein a method of preserving the imprint material and of conditioning it for use.

The binder used in preparing the material is of utmost importance. Gelatinous jellies, the consistency of which should be as high as possible,

are desirable, and I have found that class of such material, which broadly falls under the term of agar agar, the most suitable binder, provided a highly concentrated homogeneous aqueous mixture thereof can be prepared, which does not form lumps.

In the prior art commercial agar agar could not be liquefied in aqueous solution without forming lumps at a higher concentration than at an approximate agar-water ratio of 1:20.

The major object of my invention is to condition commercial agar agar in such a way that it forms a homogeneous, cohesive mixture with water at a considerably higher concentration than that mentioned above or known heretofore.

This is attained by freezing the commercial agar agar after it has been mixed with the water, or otherwise changing or destroying the cell structure thereof and releasing the readily soluble gelosine. In this manner I have obtained a homogeneous binder, which contains agar agar and water in a ratio of up to 1:6.

This novel agar solution provides a basis for many other compounds which require a high concentration of agar agar.

Such a high concentration may also be obtained by exposing the mixture to ultra-violet rays, which destroys the cellular structure of agar agar, releasing the gelosin.

As a body for a molding compound of this kind organic materials and argillaceous earth have been used most commonly heretofore. I have found the predominant use of such materials for the purpose of giving body to an imprint material to be incompatible with the objects which were mentioned above; they do not furnish a lasting material, allowing putrefaction, contraction and molding; they crack when dried; most of them cannot be restored to their original shape; and they will,—particularly argillaceous earth, bentonites, and fuller's earth,—absorb and retain air, to an extent where the negative casts made from such a material, are of an inferior quality.

The object of providing a body substance which is not subject to such short-comings has been attained by using as a major part of the body a substantially insoluble virgin rock which in itself provides for a more compact structure; still, a minor part of the body may be made up of a filler such as clays, diatomaceous-earth, fossil earth, argillaceous earth, and the like so that a material of denser structure is obtained. But the proportionate contents of the organic material or of such materials that are partly organic, are in all instances restricted to a minor proportion of the ingredients of the body, so that their disadvantages do not prevail.

The following exemplary formula may be used for explaining a simple and economic way in which this imprint material may be prepared:

|                               | Parts |
|-------------------------------|-------|
| Powdered dry agar             | 24    |
| Distilled water               | 140   |
| U. S. P. glycerine            | 18    |
| <br>Body                      |       |
| Powdered dry soapstone (rock) | 34    |
| Powdered dry zinc oxide       | 17    |
| Powdered dry silica (rock)    | 32    |
| Pulverized dry clays          | 20    |
| 15 parts E. Ball clay         |       |
| 5 parts molding clay          |       |

All ingredients of body and binder are computed  
75 "by weight".

The zinc oxide, commercial or natural (zincite), serves as a cohesive agent as well as for the purpose of closing the pores of the finished material. As coloring agent  $Fe_2O_3$  was used. The choice of coloring matter is of course arbitrary.

There are several ways to prepare this imprint material, but one of them I consider highly suitable, hygienic and economical:

(1) The liquid ingredients (water, glycerine) should be mixed at room temperature;

(2) All dry and pulverized ingredients such as commercial agar agar, stone, clays, zinc oxide (if desired, also asbestos fiber) should be weighed and mixed thoroughly with each other;

(3) Under constant but slow stirring the thoroughly mixed dry ingredients are added to the liquid (water-glycerine-solution), until a homogeneous batter has formed. Special care should be taken that no air is introduced into this batter (while and after mixing) that will happen if the stirring device rotates too fast.

(4) This homogeneous batter should be frozen in any one of the rapid-acting commercial freezers (using crushed dry-ice combined with ether, or the like). The freezing should continue even after all of the batter seems to be frozen stiff in order to assure the mutilation or destruction of substantially all agar agar cells.

(5) The frozen batter is melted and under constant slow stirring gradually heated up to the point where the agar agar mixture will begin to liquefy, and there the heating should be discontinued. (This point varies with the kinds of agar employed, but will be in the neighborhood of from 40 to 70 centigrades). This warm batter is filled into containers, preferably of the design referred to hereinafter. After introducing the batter in these containers, the latter may be sealed permanently as the further steps of the process do not require direct handling of the material. (Under certain circumstances the frozen and re-melted batter may be introduced into the containers without previous heating, although care must be taken not to bring free air into the containers as this may have a detrimental effect upon the contents therein).

(6) The containers with the material are then placed into an autoclave. This name is commonly applied to a machine much used in industrial plants for the purpose of subjecting materials to heat and pressure. Here the material is subjected for 60 minutes to a heat of  $250^{\circ}$  Fahrenheit (121° centigrade) and to not more than 15 lbs. pressure of live steam. (If the heat and the steam pressure rises above afore-mentioned limits, the characteristic quality of re-jellification of the agar agar will gradually decrease until, at a certain temperature or pressure (20 lbs.) the agar agar will cease to gelatinize). During this heating process certain important changes will take place in the material: (a) the agar agar will liquefy and combine with the water-glycerine mixture, forming later,—when cooled,—the desired highly concentrated agar-jelly; (b) the liquid agar solution will be evenly distributed throughout the whole batter inside the container, forming a fine network of agar-channels between the multi-shaped solid particles of the mixture, and I obtain a substantially homogeneous mass,—the imprint material; (c) incidentally all bacteria and spores, which might have been introduced into the mixture, will be destroyed,—leaving the material absolutely sterile until the container is opened for the purpose of using the contents for making an imprint.

Another way to manufacture the imprint material would be the following:—

The powdered dry agar agar is mixed thoroughly with the water until a stiff batter is formed in which all agar-particles have come into direct contact with the liquid. Then this batter is frozen as quickly as possible in order to prevent loss of water by evaporation. The freezing process should be continued until the greenish-gray 10 color of the agar-agar batter temporarily turns white.

Precaution should be taken that the freezing fluid does not come into direct contact with the batter as this will prevent in most cases re-jellification, and moreover, when ether contacts with the agar agar it confers upon the latter a nauseating odor and unpleasant taste.

The freezing process should be continued until the agar agar batter is thoroughly frozen and its 20 color has changed temporarily to white. The frozen cake of agar is then removed from the freezer, placed into a heating vessel equipped with a slowly rotating stirring device, and covered with so much glycerine as the ultimate use of the material may warrant. This treatment serves two-fold: First, while the frozen agar is melting the layer of glycerine prevents loss of water by evaporation; second, due to the slow melting of the frozen agar and the constant stirring, the glycerine will be thoroughly and finely distributed throughout the whole agar solution. Direct application of heat up to the boiling point will finally yield a highly concentrated homogeneous agar solution of the afore-mentioned ratio.

35 This novel agar solution furnishes a basis for many compounds which require a high concentration of agar agar.

From this stage I proceed as follows to obtain the imprint material:

40 The frozen agar agar, as it was covered with glycerine, is melted, heated under constant stirring, and likewise under constant stirring the dry and powdered ingredients are added until thoroughly mixed with the agar-water-glycerine mixture, forming a stiff batter of high consistency. The heating temperature is raised up to 100 centigrade, and kept at the boiling point for a short period.

50 The mixture is now filled into containers and sealed.

There is another method whereby the highly concentrated agar solution may be obtained:

Again the dry agar agar and water are thoroughly mixed and then irradiated with ultra-violet rays. Such ultra-violet treatment will destroy the cellular structure lower the absorption capacity of agar agar to considerable extent and by releasing the soluble gelatin lower the dissolving temperature of agar agar to about 40 centigrade, permitting thereby much higher concentration than heretofore has been possible. Due to the fact that certain agar agars are less resistant to ultra-violet rays than others, the irradiation period should,—generally,—not exceed 30 minutes. Excessive irradiation may result in partial or complete loss of the agar agar's characteristic quality of being liquefied and solidified repeatedly, without detrimental influences. After 60 treatment of the agar agar with ultra-violet rays an imprint material is prepared exactly as described in connection with the previously described processes after freezing and thawing.

In order to increase the cohesion in such concentrated agar agar solutions commercial or

natural zinc oxide (zincite) (up to 15% of the body-forming ingredients) may be added to and incorporated in the mixture in finest distribution.

To increase elasticity and likewise to absorb surplus water, non-frozen powdered dry agar agar may be added additionally in small quantities (up to 2%). The tiny cells of the agar agar possess high absorption power (about 20 times their dry-weight) and besides are valuable for the reconstruction of the dried-out and shrunk materials to their former original dimensions and shape.

In accordance with the intended use of the material, certain modifications of the basic formula may be brought about, which may be guided by the following considerations:

The necessary concentration of agar agar may be reduced by substituting substances of more tenacious and mucilaginous character such as gelatin (glue of bones), Moussé de Chine, Layor 20 Caranga, algae of the *rhodophyceae*-specie, or isinglass and the like, resulting in an imprint material of high viscosity but slower setting speed.

An increase of the glycerine contents,—with 25 or without a proportionate decrease in water,—will give a fatty, slow-drying material, which, when air-dried possesses leather-like appearance of rather tough and tenacious character—but the material will also mold more readily. 30

Increasing the silica-rock and decreasing the clay contents, will result in a more porous and faster drying material, but it is also apt to crack while a cast dries.

Replacing part or the whole of the natural 35 rock ingredients in the mixture by commercially improved silica such as calcined diatomaceous silica or calcined fossil silica will result in a material of extremely light weight as may be desired for taking delicate imprints of such objects as hair.

A suitable formula is:

| Binder                    | Parts |
|---------------------------|-------|
| Dry powdered agar agar    | 20 45 |
| Distilled water           | 140   |
| Glycerine                 | 10    |
| Body                      |       |
| Silica ash                | 30    |
| Powdered SiO <sub>2</sub> | 50    |
| Zinc oxide                | 20    |
| South Carolina clay       | 10    |

Generally, the calcined silica may be added in a quantity sufficient to impose upon the imprint material a characteristic compactness, lightness and yieldability, lightness in color too, unless offset by coloring ingredients. In the foregoing the SiO<sub>2</sub> and clay may also be replaced by calcined silica also termed silica ash.

For purposes of this invention calcined silica 60 should therefore be classified as a "rock".

An introduction of asbestos fiber into the material will provide structure and tensile strength in the compound as a whole, but not more than 3% of the entire weight of ingredients in the 65 imprint material should be added. Long fibers have a tendency "to coil up" in the mixture forming annoying lumps, and likewise may impair the detail of the imprint. In order to increase the tensile strength it is advisable to use raw, 70 crude asbestos fiber in preference to commercially improved fiber.

If material of less consistency is desired, the agar water proportion may be stretched, although the glycerine should be increased in proportion; 75

due to the lessened amount of the agar binder in such a material another cohesion-increasing agent should be introduced in the material to make up for the loss in binding power.

5 Exceedingly fine-grained clays produce sharper imprints, but may lose in detail if immersed in cold water and may also color the saliva,—if used for dental purposes.

Darker clays are more fatty, than light-colored ones; the former will ordinarily retain water and moisture longer than the latter, but they dry slower and invite bacterial growth.

10 Bentonite clays absorb about 12 times their weight in water and increase in volume considerably while doing so, but upon drying they shrink extremely and crack the cast due to their abnormal shrinkage; besides, bentonites have a tendency to absorb and retain air, which may give the material large voids and a sponge-like 15 appearance, which is very annoying if detail is wanted.

13 The term agar agar is used here to describe certain material which has certain physical characteristics. The derivates of agar agar, gelose for instance or any other equivalent compound 20 may be substituted wholly or partly for the agar agar.

18 Agar agar is very sensitive to acids, and in the choice of rocks, earth, and organic material, care 25 should be taken that such material is not acidic.

In order to illustrate modifications, for instance for the purpose of introducing a higher silica content, I also give the following exemplary formula:

|                         | Parts |
|-------------------------|-------|
| Binder                  |       |
| Powdered dry agar       | 23    |
| Distilled water         | 140   |
| U. S. P. glycerine      | 10    |
| Body                    |       |
| Powdered $\text{SiO}_2$ | 60    |
| Powdered soapstone      | 24    |
| Dry South Carolina clay | 22    |
| Zinc oxide              | 16    |

45 I may go to the point of eliminating argillaceous earth and clays altogether, in which instance the following exemplary formula may be adhered to in preparing my material as described before:

|                    | Parts |
|--------------------|-------|
| Distilled water    | 140   |
| Powdered agar agar | 20    |
| U. S. P. glycerine | 10    |

55 To that mixture, after freezing and melting, add:

|                                    | Parts |
|------------------------------------|-------|
| Powdered soapstone (200 mesh)      | 42    |
| Powdered $\text{SiO}_2$ (140 mesh) | 36    |
| Powdered quartz (flint, 200 mesh)  | 20    |
| Zinc oxide                         | 20    |
| Dry powdered agar agar (Jap.)      | 4     |

65 Proceeding in accordance with the second manufacturing method described above, the material is substantially finished, when it is placed into a container and sealed therein; any type of a closure, a can for instance, which can be sealed or closed air tight, is suitable.

70 But in the first method referred to, the material is subjected to further treatments after having been sealed in the container, and, since these comprise heat and pressure treatments in which the material changes in volume, and since it is not advisable to allow the amount of air necessary for a cushion in the container, the container

should be collapsible and readily allow propagation of pressure and heat therethrough and throughout the contents. Therefore I prefer the use of a flattened container, made of thin-sheet metal or other yieldable material.

Such a container is illustrated in the accompanying drawing, in which:

Fig. 1 shows a perspective view of the closed container;

Fig. 2 shows a longitudinal section thereof. 10

Fig. 3 is a cross-section.

In the drawing, the collapsible tube 11 is the flat body of the container; the ends 12 are folded over, and sealed and the container is filled with the material.

15 These metal containers are filled with the imprint material,—not to the amount they could receive when shaped cylindrically, but to their capacity in the flat condition shown,—closed and sealed permanently. Turning the ends of 20 the collapsible tube over flat, will also allow for expansion during heat treatments. In this state, the metal containers and the material therein enclosed are subjected to the heat and pressure specified above.

25 The material, in a sealed container of the type shown, may be kept indefinitely. When to be used, its temperature is raised to about 60° centigrade in boiling water, whereupon one end of the container is clipped off and the material 30 squeezed out of the container and then used to take the imprint. It will set in one or two minutes (according to its consistency and ingredients) and then the imprint may be withdrawn from the article from which the imprint 35 was taken. The material will preserve its original size for about one-half of one hour or more, and then, in the period of days according to climatic conditions will shrink as it loses moisture. A shrunken, and dried out, imprint may 40 be reproduced to true imprint size at any time by being soaked in plain water or in water with a trace of glycerine. This soaking should extend from a few minutes up to about 24 hours,—depending upon the grade of desiccation of the cast. 45

Freshly made imprints may be preserved for days and weeks in their exact shape and size, without shrinkage, by keeping them in an airtight container, such as a glass jar with fitted-in stopper. A few drops of distilled water keeps 50 the air moist inside of this container, and a drop of phenol, formaldehyde (formalin) or the like should be added to prevent bacterial growth.

55 Although I have shown and described one form of embodiment of my invention in detail, yet I do not wish to be limited thereby, except as the state of the art and the appended claims may require, for it is obvious that various modifications and changes may be made in the form of embodiment of my invention, without departing from the spirit and scope thereof.

60 What I claim is:—

1. An imprint material comprising a highly concentrated homogeneous gelatinous binder, a body of powdered material and a mixture of hard and soft virgin rock forming the major part of said body material.

2. In an imprint material a homogeneous gelatinous binder comprising agar agar and water, at a ratio exceeding 1 to 7.

3. The method of preparing a homogeneous binder of an imprint material containing a high concentration of agar agar in water, comprising mixing agar agar into water, irradiating said 75

mixture with ultra-violet rays, and heating it until it forms a gel.

4. The method of preparing an imprint material with an agar agar binder and a mineral body, comprising rapidly freezing an agar agar-water-glycerine batter, and boiling said solution with a mineral body in powdered form.

5. An agar agar solution characterized by a high concentration of agar agar and water, said solution being a homogeneous gel containing agar agar and water of substantially the ratio 1 part agar agar to 6 parts of water and obtained by heating a non-gelatinous mixture of agar agar and water, after the cellular structure of the agar agar in said mixture has been broken up so that the gelatin in the cells is set free.

6. A highly concentrated agar agar solution obtained by rapidly freezing a substantially non-gelatinous mixture of agar agar and water, and later heating said mixture to the point where the agar agar dissolves.

7. An agar agar solution, characterized by a concentration of agar agar in water in excess of a proportion of 1:7, prepared by rapidly freezing a substantially non-gelatinous agar agar-water mixture, and then heating said mixture to the point where the agar agar dissolves.

8. The method of preparing an imprint material, comprising mixing a batter of agar agar and cold water in high concentration, irradiating said mixture with ultra-violet rays for a prede-

termined period, heating the mixture until it dissolves, and adding a powdered body material thereto.

9. A substantially non-shrinking imprint material comprising a concentrated agar agar water gel of the type described in claim 5 and powdered rock.

10. In an imprint material a binder comprising a viscous homogeneous mixture containing agar agar and water substantially in the ratio of 1 part agar agar to approximately 6 parts by weight of water.

11. The method of preparing a homogeneous binder for an imprint material containing a highly concentrated emulsion of agar agar in water, comprising mixing agar agar and cold water, rapidly freezing the mixture, and heating said mixture to the point where the agar agar dissolves.

12. The method of preparing an imprint material, comprising the preparation of a cold mixture of commercial agar agar, water, and the required mineral substances, freezing said mixture, melting said frozen mixture and heating it until a highly concentrated paste is obtained.

13. A highly concentrated agar agar solution prepared from a frozen non-gelatinous substantially 1:6 mixture of agar agar and water.

HENRY VON BRANDT. 30